

## 1

2,725,345

## STABILIZED MINERAL OILS AND METHOD OF PREPARATION

Kurt Binovic, Boulogne, and Robert Dupas, Notre Dame de Gravenchon, France, assignors to Esso Standard Societe Anonyme Francaise, Paris, France, a body corporate

No Drawing. Application February 19, 1952,  
Serial No. 272,516

Claims priority, application France February 21, 1951

## 9 Claims. (Cl. 196—151)

The present invention relates to stabilized mineral oils and a method for improving the stability to oxidation of mineral oils, and more especially those mineral oils which have been refined with sulphuric acid or oleum.

It is known that the refining of mineral oils, particularly insulating oils and certain turbine oils, requires a more or less severe treatment with sulphuric acid to give them certain desirable qualities among which is good stability during service.

Experience has proved, however, that there is an optimum treatment beyond which the stability diminishes, i. e. beyond which the acid index increases too rapidly in use. It results from this that if a severe sulphuric acid treatment is necessitated by the color or insoluble deposits, the oil obtained is insufficiently stable, particularly as regards the development of acidic products and consequent increase in the acid index during service.

To obviate this, it has often been advocated to add to oils of low stability to oxidation, different fractions of petroleum in proportions varying between 10 and 50%. In this way there has been advocated, with the object of increasing the stability to oxidation of mineral oils, the use of unfinished cylinder oils or "Bright stock" or different solvent extracts, obtained from medium fractions of petroleum, after-treated with acid or activated earth.

The addition of large proportions of other petroleum fractions to finished oils frequently may be very inconvenient. In particular, in the case of special highly refined oils for which the improvement obtained is made to the detriment of other qualities the properties of the oil, such as viscosity, flash and freezing point, may even be completely changed. Moreover, the expenses of adding large proportions of other petroleum fractions may prevent the economic use of this method of stabilizing mineral oils. On the other hand, the addition of relatively very small quantities of other fractions is not objectionable though commonly considered ineffective.

It has now been discovered that the stability of mineral oils to oxidation can be improved by the addition of up to 1% by volume of a heavy oil fraction obtained by deasphalting a heavy residual oil from the distillation of crude petroleum. The invention is applicable to mineral oils generally but particularly to those fractions of moderate viscosity, i. e., of the insulating oil-lubricating oil range.

The heavy residual oil may be obtained as the residue on distilling crude petroleum under vacuum. The deasphalting of the residual oil may be carried out by known means, preferably by the use of propane.

The deasphalted heavy oil residuum is preferably used for purposes of the present invention in amounts of between 0.1 and 1% by volume of the mineral oil to be stabilized. Proportions as low as 0.01% may be used for some purposes.

It has also been discovered that even more pronounced stabilizing effects are produced by treating the deasphalt-

## 2

ised heavy oil residual oils with a selective solvent such as phenol, furfural or preferably tetrahydrofurfuryl alcohol.

The antioxidant effect of the deasphalted heavy residual oil and of the fractions obtained from such deasphalted heavy residual oils by different treatments have been tested on a mineral insulating oil, obtained by the sulphuric acid refining of a light distillate from a Coastal crude.

The characteristics of the insulating oil which was treated were as follows:

|                            |             |
|----------------------------|-------------|
| Density at 15° C.          | 0.885       |
| Engler viscosity at 20° C. | 4.69        |
| Flash (Cleveland)          | 164/182° C. |
| Tag-Robinson color         | 24          |
| Thomson tar                | 0.016       |
| Freezing point             | —48° C.     |
| Acid index                 | 0.01        |

The oxidation tests were carried out according to the "Staeger Life Test," slightly modified.

The oil or mixture of oils (200 cc.) was oxidized in an oven with a revolving floor (4-6 R. P. M.) at  $110^{\circ} \pm 0.5^{\circ}$  C., a current of purified air at 47-54 litres per hour passing through the oven, and in presence of plates of polished electrolytic copper of 40x70x0.1 mm. replaced every 72 hours.

Samples of .20 gm. of oil were taken after 72, 144 and 192 hours of oxidation and the acid index was measured. The color (Tag-Robinson) was measured after 192 hours. The acid index and color were measured before the oxidation.

Measurements of stability were also carried out according to the method of the Brown Boveri Company, as shown below.

There will be given hereafter examples, in no way limiting, which will better illustrate the features of the invention.

## Example I

A petroleum from Arabia (Aramco) was distilled under vacuum until only 14% of residue was left. This latter was taken up in 800% by volume of propane and allowed to separate at 45° C. After separation of the asphalt, the upper layer was collected and the propane separated by distillation. There was thus obtained 8% of a very viscous oil.

0.1% of this deasphalted residue was added to the insulating oil described above.

This mixture and the insulating oil without addition were submitted to oxidation according to the modified Staeger Life Tests.

The results obtained were as follows:

| 60 | Composition                                                         | Acid Index in mg. KOH per gm. oil |                  |                      |                      | Tag-Robinson Color       |                      |
|----|---------------------------------------------------------------------|-----------------------------------|------------------|----------------------|----------------------|--------------------------|----------------------|
|    |                                                                     | Before Oxida-<br>tion             | After<br>72 Hrs. | After<br>144<br>Hrs. | After<br>192<br>Hrs. | Before<br>Oxida-<br>tion | After<br>192<br>Hrs. |
| 65 | Insulating Oil                                                      | 0                                 | 0.04             | 0.18                 | 0.31                 | 24                       | 4                    |
|    | Insulating Oil +<br>0.1% Deasphal-<br>tised Heavy Re-<br>sidual Oil | 0                                 | 0.018            | 0.07                 | 0.125                | 20 <sup>1/2</sup>        | 8                    |

The insulating oil and its mixture with 0.1% of deasphalted residual oil stock were also oxidized according to the method of the Brown Boveri Company.

The results were as follows:

| Composition                                                     | Acid Index mg. KOH per gm. oil |                  |                   |                  | Insoluble Deposit |                  | Decrease In Strength Of Cotton |  |
|-----------------------------------------------------------------|--------------------------------|------------------|-------------------|------------------|-------------------|------------------|--------------------------------|--|
|                                                                 | Before Oxida-<br>tion          | After 72<br>Hrs. | After 168<br>Hrs. | After 72<br>Hrs. | After 168<br>Hrs. | After 72<br>Hrs. | After 168<br>Hrs.              |  |
| Insulating Oil.....                                             | 0                              | 0.056            | 0.28              | 0.002            | 0.042             | 30               | 50                             |  |
| Insulating Oil+0.1% De-<br>asphalted Heavy Residual<br>Oil..... | 0                              | 0.042            | 0.155             | None             | 0.03              | 27               | 32                             |  |

### Example II

The deasphalted heavy residual oil stock, obtained as indicated in Example I was treated with 400% of phenol in countercurrent at 70° C. The upper phenol-free layer (raffinate) was then added in an amount of 0.1% by volume to the insulating oil, and this mixture and the pure insulating oil were oxidized according to the modified Staeger Life Test.

The results obtained were as follows:

| Composition                            | Acid Index in mg. KOH per gm. oil |                 |                  |                  | Tag-Robinson Color    |                   |
|----------------------------------------|-----------------------------------|-----------------|------------------|------------------|-----------------------|-------------------|
|                                        | Before Oxida-<br>tion             | After 72<br>Hr. | After 144<br>Hr. | After 192<br>Hr. | Before Oxida-<br>tion | After 192<br>Hrs. |
| Insulating Oil.....                    | 0                                 | 0.04            | 0.18             | 0.31             | 24                    | 4                 |
| Insulating Oil+<br>0.1% Raffinate..... | 0                                 | 0.02            | 0.08             | 0.15             | 22                    | 8½                |

The same trials carried out according to the Brown Boveri Company test had the following results:

| Composition                             | Acid Index mg. KOH per gm. Oil |                 |                  |                 | Insoluble Deposit |                 | Decrease In Strength Of Cotton |  |
|-----------------------------------------|--------------------------------|-----------------|------------------|-----------------|-------------------|-----------------|--------------------------------|--|
|                                         | Before Oxida-<br>tion          | After 72<br>Hr. | After 168<br>Hr. | After 72<br>Hr. | After 168<br>Hr.  | After 72<br>Hr. | After 168<br>Hr.               |  |
| Insulating Oil.....                     | 0                              | 0.056           | 0.28             | 0.002           | 0.042             | 30              | 50                             |  |
| Insulating Oil+0.1% Raffi-<br>nate..... | 0                              | 0.042           | 0.15             | None            | 0.015             | 10              | 40                             |  |

### Example III

The deasphalted heavy residual oil stock, obtained as described in Example I, was treated with 100% of tetrahydrofurfuryl alcohol at room temperature. After some hours of decantation, the two layers were separated.

The lower layer (extract) was freed from tetrahydrofurfuryl alcohol by distillation. The fraction so obtained was added in an amount of 0.4% by volume to the insulating oil. This oil and the mixture were submitted to oxidation according to the modified Staeger Life Test.

The results were as follows:

| Composition                                                              | Acid Index in mg. KOH per gm. Oil |                 |                  |                  | Tag-Robinson Color    |                  |
|--------------------------------------------------------------------------|-----------------------------------|-----------------|------------------|------------------|-----------------------|------------------|
|                                                                          | Before Oxida-<br>tion             | After 72<br>Hr. | After 144<br>Hr. | After 192<br>Hr. | Before Oxida-<br>tion | After 192<br>Hr. |
| Insulating Oil.....                                                      | 0                                 | 0.04            | 0.18             | 0.31             | 24                    | 4                |
| Insulating Oil+<br>0.4% Extract By<br>Tetrahydrofurfuryl<br>Alcohol..... | 0                                 | 0.035           | 0.055            | 0.07             | 16                    | 4½               |

It may be seen from these results that the addition of deasphalted heavy residual oil stocks to mineral oils

increase their stability as indicated by substantial reductions in the amounts of organic acids and insoluble deposits formed during service. Moreover, the color is seen to be improved slightly after oxidation.

Solvent treatment of the deasphalted heavy residual oils with tetrahydrofurfuryl alcohol is seen to improve the stability of mineral oils to which they are added, even more.

What is claimed is:

1. An oil composition of high oxidation resistance comprising a mineral base oil fraction of insulating-lubricating oil viscosity grade containing 0.01 up to 1% by volume of a propane deasphalted residual oil from the distillation of crude petroleum.

2. Composition as claimed in claim 1 wherein there is present from 0.1 to 1% by volume of the deasphalted residual oil.

3. Compositions as claimed in claim 2 wherein the deasphalted residual oil is first subjected to a selective solvent extraction treatment.

4. Composition as claimed in claim 3 wherein the solvent used is tetrahydrofurfuryl alcohol.

5. Compositions as claimed in claim 3 wherein the solvent used is phenol.

6. A method of stabilizing mineral oils of insulating-lubricating oil viscosity range against oxidative deterioration comprising adding between 0.01 and 1% of a propane deasphalted residual oil from the distillation of crude petroleum.

7. A method as claimed in claim 6 wherein the deasphalted residual oil is first subjected to a selective solvent extraction treatment.

8. A method as claimed in claim 6 wherein the deasphalted residual oil is first subjected to a selective solvent extraction treatment with tetrahydrofurfuryl alcohol.

9. A method as claimed in claim 6 wherein the deasphalted residual oil is first subjected to a selective solvent extraction treatment with phenol.

### UNITED STATES PATENTS

References Cited in the file of this patent

|    |           |                |               |
|----|-----------|----------------|---------------|
| 70 | 1,833,374 | Hill           | Oct. 18, 1932 |
|    | 2,117,602 | Bulkley        | May 17, 1938  |
|    | 2,139,668 | Breth et al.   | Dec. 13, 1938 |
|    | 2,165,432 | Whiteley       | July 11, 1939 |
|    | 2,195,659 | Shoemaker      | Apr. 2, 1940  |
|    | 2,200,534 | Bray           | May 14, 1940  |
| 75 | 2,295,035 | Gilbert et al. | Sept. 2, 1942 |